

Patented May 11, 1926.

## UNITED STATES PATENT OFFICE.

WILLIAM E. DAY, JR., OF NEW BRUNSWICK, NEW JERSEY, ASSIGNOR TO INTERNATIONAL MOTOR COMPANY, OF NEW YORK, N. Y., A CORPORATION OF DELAWARE.

## HIGH LEAD-BRONZE ALLOY AND METHOD OF MANUFACTURING THE SAME.

No Drawing. Application filed October 20, 1923. Serial No. 669,709.

This invention relates to an alloy which possesses high bearing qualities and will run for long periods without lubrication and without causing any cutting of the shaft 5 or other element journaled therein, and the method of so manufacturing the same as to insure the desired physical properties.

While it will be understood that some latitude is to be allowed to one skilled in the art in the percentages employed with respect to the main ingredients and also as to the temperature employed and the technique used it has been found in practice that an alloy of high lead bronze comprising, in general, the following ingredients will satisfy the requirements of use:

Lead 20-25%, tin 7-10% and the balance copper.

The amount of tin, in general, will depend on the hardness desired.

In the course of manufacturing a deoxidizer is employed and this, of course, carries small amounts of nickel, zinc and phosphorus, or other elements into the main ingredients.

The preferred method employed in the manufacture of the compound is to melt down the copper and then add the lead and bring the whole to 2700° F. It has been found that by raising the mixture to a temperature approaching or perhaps exceeding the boiling point of lead, the lead tends to assume a very finely divided state approaching almost a colloidal condition, and to become evenly dispersed throughout the alloy. This condition is preserved more or less in the alloy after solidification. The tin is then added, and a small quantity of a suitable deoxidizer, consisting, for instance, of zinc, nickel, copper and phosphorus, is added to the extent of approximately two percent (2%) of the entire mass. About

one percent (1%) more of this deoxidizer is placed in the bottom of a hot pouring ladle and the metal from the furnace is then poured in the ladle. The mixture is then thoroughly stirred and the dross skimmed from the top after which it is poured in molds. After the alloy has been made by heating to a temperature of substantially 2700° F. the temperature of the mass may be permitted to drop to temperature suitable for pouring.

As indicated hereinbefore the alloy thus formed possesses high bearing qualities, requires little lubrication and will not cut the element journaled therein. Ordinary departures with respect to the ingredients and method of manufacture may be resorted to by one skilled in the art without avoiding the substance of the invention.

## What I claim is:

1. The herein described method of manufacturing a bearing alloy consisting in combining lead and copper and bringing the whole to at least 2700° F., then adding tin and a small quantity of a deoxidizer, pouring the mass into a hot pouring ladle, and introducing the metal into molds.

2. The herein described method of manufacturing a bearing alloy consisting in melting down copper, adding lead, bringing the whole to 2700° F., then adding tin and a small quantity of a deoxidizer consisting of zinc, nickel, copper and phosphorus to the amount of approximately two percent of the entire mass, pouring the metal into a hot ladle containing one percent more of the deoxidizer skimming and introducing the alloy into molds.

This specification signed this 16 day of Oct. A. D. 1923.

WILLIAM E. DAY, JR.